# EUROPEAN PATENT SPECIFICATION

(11) **EP 4 020 505 B1**
(45) Date of publication and mention of the grant of the patent: **12.07.2023**
(21) Application number: 21214513.0
(22) Date of filing: 14.12.2021
(51) Int. Cl.: H01F 41/02, H01F 1/057

(54) **PREPARATION METHOD FOR A NEODYMIUM-IRON-BORON MAGNET**
VERFAHREN ZUR HERSTELLUNG EINES NEODYM-EISEN-BOR-MAGNETEN
PROCÉDÉ DE PRÉPARATION D'UN AIMANT NÉODYME-FER-BORE

(30) Priority: 15.12.2020 CN 202011473669
(43) Date of publication of application: 29.06.2022
(73) Proprietor: Yantai Dongxing Magnetic Materials Inc., 265500 Yantai City (CN)
(72) Inventor: Zhu, Xiaonan, Yantai City, 265500 (CN); Peng, Zhongjie, Yantai City, 265500 (CN); Xiang, Chunjie, Yantai City, 265500 (CN); Zhang, Qiang, Yantai City, 265500 (CN); Ding, Kaihong, Yantai City, 265500 (CN)
(74) Representative: Gulde & Partner

(56) References cited:
- EP-A2- 1 793 392
- WO-A1-2015/096583
- CN-B- 103 106 991
- US-A1- 2015 243 416
- US-A1- 2015 248 954

## Description

### BACKGROUND OF THE INVENTION

### Field of the Invention

The present disclosure relates to a method for preparing magnetic materials, in particular for preparing a sintered NdFeB magnets.

### Description of the Prior Art

Permanent magnet materials are the most widely used, and rare earth permanent magnet is an important part of permanent magnet materials, especially the third generation of rare earth permanent magnet NdFeB permanent magnet material has been widely used with its excellent magnetic properties.

With the further expansion of application fields, higher requirements are put forward for the performance of NdFeB permanent magnet materials. In order to meet the requirements of operating temperature in applications such as motors and generators, it is necessary to increase the maximum operating temperature of sintered NdFeB. The main ways include increasing the Curie temperature, coercivity and magnetocrystalline anisotropy field. Studies have shown that adding heavy rare earth elements, such as Dy and Tb, to the magnet is the most effective means to improve the magnet's working temperature and coercivity. Due to the low reserves and high price of heavy rare earth elements, the addition increases the cost of the magnet. At the same time, due to the anti-ferromagnetic coupling between heavy rare earth and iron, the heavy rare earth Dy and Tb element was entered into the main phase by smelting alloy, and reduced the remanence of the magnet.

How to increase the coercivity of the magnet without reducing the remanence and the low content of heavy rare earths has become an urgent problem in the development of neodymium iron boron permanent magnets.

At present, the most effective way to increase the coercivity is to improve the grain boundaries and diffuse low amount of Dy and Tb into the main phase. The clear continuous grain boundary phase inhibits the nucleation of anti-magnetization domains and improves the coercivity while avoiding the decline of remanence. Due to the limitation of the diffusion depth of grain boundary, it is only suitable for magnets with thickness less than 5mm. In addition, the low utilization rate of heavy rare earth will also increase the production cost. Patent number ZL201110242847.7 invented a preparation method of low Dy content and high performance sintered NdFeB. The Dy element is introduced into the particle surface of powder by sputtering deposition method that Dy element is difficult to accurately control. Patent number CN109102976 invented a method to improve the performance of rare earth magnet, with heavy rare earth alloy adding into the main grain boundary and the heavy rare earth distributing to the main phase boundary. It is not only reducing the milling efficiency and increasing the risk of nitride and oxide, but also reducing the efficiency of magnet production, for the production of grain refinement process and low temperature sintering process for a long time.

US 2015/248954 A1 discloses a method of manufacturing an NdFeB sintered magnet by mixing light rare earth based and heavy rare earth based alloys, further supplemented with a Dy₂O₃ micro-powder, to form an NdFeB sintered magnet by magnetic field pressing, sintering and ageing.

### SUMMARY OF INVENTION

The present invention provides a preparation method for a NdFeB permanent magnet as defined in claim 1. The method includes the steps of:
a) Preparing main alloy flakes consisting of (Pr₂Nd₈)ₓFe_{100-x-y-z}B_{y}M_{z}, where M is at least one of Al, Co, Cu, Ga, Ti and Zr, and x, y and z is 28.5wt.%≤x≤31.0wt.%, 0.85wt.%≤y≤0.98 wt.% and 0.5wt.%≤z≤5.0wt.%;
b) Preparing auxiliary alloy flakes consisting of LᵤFe_{100-u-v-w}BᵥM_{w}, where L is one or more of the metals Pr and Nd, M is at least one of Al, Co, Cu, Ga, Ti and Zr, and u, v and w is 35.0wt.%≤u≤45.0wt.%, 0wt.%≤v≤5.0wt.% and 2.0wt.%≤w≤10.0wt.%;
c) Mixing the main alloy flakes and the auxiliary alloy flakes in a predetermined rate, then performing a hydrogen decrepitation to produce alloy pieces, and then crushing the alloy pieces to an alloy powder by jet milling;
d) Preparing a powder mixture including the alloy powder and an added heavy rare earth powder consisting of at least one of Dy and Tb; and
e) Pressing the powder mixture to a green compact while applying a magnetic field, and thermal treatment of the green compact in a vacuum furnace to obtain the NdFeB permanent magnet.

According to one embodiment, the auxiliary alloy may include Pr and Nd. In particular, a content ratio of Pr to Nd may be in the range of 0.25 to 1.

According to another embodiment, which could be combined with the before mentioned embodiment, the auxiliary alloy flakes are added in proportion of 5wt% to 20wt% in step c). According to another embodiment, which could be combined with one or more of the before mentioned embodiments, the heavy rare earth powder, which is added in step d), has an average particle size D50 in the range of 1.0µm to 3.0µm, the mass percentage of the heavy rare earth is in the range of 0.05wt.% to 1.0wt.%, and the powder are mixed about 90-150min.

According to another embodiment, which could be combined with one or more of the before mentioned embodiments, the thermal treatment of step e) includes a sub-step of sintering the green compact at a temperature in the range of 850°C to 950°C for 2 to 5 hours, and then heating to 1030°C to 1090°C for 4 to 8h. Furthermore, the thermal treatment of step e) may further include the sub-steps of cooling the sintered green compact, and then annealing the sintered compact at a temperature in the range of 800°C to 900°C for 2 to 4 hours and then at a temperature in the range of 450°C to 550°C for 3 to 6 hours.

It has been found by the invetors that a low melting point alloy containing no heavy rare earth could be used to transport heavy rare earth powder around the main phase. The auxiliary phase facilitates the diffusion of heavy rare earths into the main phase during the sintering process, promotes the formation of a high H_{A} phase shell layer in the main phase, and improves the coercivity.

The invention adopts the principle of diffusion, adding heavy rare earth powder (containing or consisting of Dy and/or Tb) to a NdFeB alloy containing a low melting point auxiliary phase alloy. The heavy rare earth powder is evenly dispersed around the main phase in the sintering process.

The sintering process may be divided in two sub-steps of first holding the temperature for 2 to 5h at 850°C to 950°C and then sintering at a higher temperature. Under the higher temperature, the heavy rare earth metals Dy or Tb will diffuse into the magnet and enter the surface layer of the main phase particles, forming a DyFeB or TbFeB with high H_{A}. The auxiliary alloy is easy to form the grain boundary phase with uniform continuous distribution, which will increase the coercivity during the annealing process.

### DETAILED DESCRIPTION OF THE INVENTION

The following disclosure provides a preparation method for a sintered NdFeB magnet having of high remanence and high coercivity by adding a low amount of a heavy rare earth metal.

Only a low amount of a heavy rare earth powder (Dy and/or Tb) is added during the preparation of the sintered NdFeB magnet. A low melting alloy without heavy rare earth metals is added for forming the grain boundary phase and then the heavy rare earth powder with a mass percentage in the range of 0.05wt.% to 1.0wt.% based on the total weight of the composition. According to an embodiment, the method includes the following steps:
a) Main alloy flakes are provided. The composition of the main alloy flakes is set to (Pr₂Nd₈)ₓFe_{100-x-y-z}B_{y}M_{z}, where M is at least one of Al, Co, Cu, Ga, Ti and Zr, and x, y and z is 28.5wt.%≤x≤31.0wt.%, 0.85wt.%≤y≤0.98wt.% and 0.5wt.%≤z≤5.0wt.%. The main alloy flakes do not contain α-Fe and the elements Dy or Tb.
b) Further, auxiliary alloy flakes are provided. The composition of the auxiliary alloy flakes can be set to LᵤFe_{100-u-v-w}BᵥM_{w}, where L is one or more of the metals Pr and Nd, M is at least one of Al, Co, Cu, Ga, Ti and Zr, and u, v and w is 35.0wt.%≤u≤45.0wt.%, 0wt.%≤v≤5.0wt.% and 2.0wt.%≤w≤10.0wt.%.
c) The main alloy flakes and the auxiliary alloy flakes are mixed in an appropriate rate and then a hydrogen decrepitation is performed to produce smaller alloy pieces. The alloy pieces are pulverized to an alloy powder by jet milling.
d) A powder of the heavy rare earth elements Dy or Tb is added to the jet milled alloy powder of step c). The amount of the added heavy rare earth powder is in the range of 0.05wt% to 1.0wt% and the resulting powder mixuture is mixed to uniformity using a mixer equiptment.
e) The final alloy powder obtained by step d) is pressed to a green compact while applying a magnetic field. The green compact is pit into a vacuum furnace for thermal treatment, i.e. sintering and annealing the green compact to a sintered NdFeB magnet.

In step b), when Pr and Nd metal are both selected as a rare earth element L in the auxiliary alloy, the content ratio of Pr and Nd is 0.25 to 1. In other words, the auxiliary alloy may then include 4 times as much Pr than Nd (by weight) to equal amounts of Pr and Nd, but no excess of Nd.

The main alloy flakes and the auxiliary alloy flakes are mixed in step c). The resulting mixture shall include 5wt% to 20wt% of the auxiliary alloy flakes, i.e. the main alloy flakes represent 80wt% to 95wt% of said mixture.

In step d) a heavy rare earth powder is added, especially a Dy or Tb powder. An average particle size D50 of the heavy rare earth powder may be in the range 1.0µm to 3.0µm. The average particle diameter of the particles may be for example measured by a laser diffraction device using appropriate particle size standards. Specifically, the laser diffraction device is used to determine the particle diameter distribution of the particles, and this particle distribution is used to calculate the arithmetic average of particle diameters. More precisely, the particle size of a non-spherical particle may be determined by a dynamic light-scattering measurement method. Specifically, the size may be measured by ISO 13320 through the analysis of the light-scattering properties of the particles.

Further, a mass percentage of the addded heavy rare earth powder may be in the range of 0.05wt.% to 1.0wt.%. The powders may be mixed about 90 to 150min to obtain a final alloy powder.

In step e), the final alloy powder is pressed to a green compact while applying a magnetic field of 1.8 to 2.5T. The green compact is put into a vacuum furnace to perfom a sintering and annealing process. During the sintering process, the temperature is in the range of 850°C to 950°C for 2 to 5 hours and then raised to 1030°C to1090°C for 4 to 8h. After cooling, the annealing process follows. The sintered green compact ist first heated to a temperature in the range of 800°C to 900°C for 2 to 4 hours, and then the temperature is set to be in the range of 450°C to 500°C for 3 to 6 hours.

The following technical advantages may result by performing the preparation process as described above:
The invention adopts the principle of diffusion for reference, adding heavy rare earth Dy or Tb powder to NdFeB alloy containing low melting point auxiliary phase alloy,

The heavy rare earth elements are carried by the auxiliary alloy havin a lower melting point and evenly dispersed around the main phase in the sintering process. The Dy or Tb will diffuse into the magnet and enter the surface layer of the main phase particles, forming DyFeB or TbFeB phases with high H_{A}. The coercivity is significantly improved while the remanence is not or only slightly reduced. The preparation process of magnets may be performed with reduced energy consumption and improved production efficiency compared to convential processes.

In other words, a low melting auxiliary alloy without heavy rare earth content and a small amount of heavy rare earth Dy or Tb powders is added to the main alloy powder. The grain boundary phase formed by the auxiliary alloy having a lower melting point than the main alloy forms a high-fluidity phase carrying the heavy rare earth Dy or Tb distribution around the main phase of the main alloy. In the process of sintering, the heavy rare earth Dy or Tb powders diffuse into the surface of the main phase to realize the introduction of heavy rare earth elements. The auxiliary alloy is easy to form the grain boundary phase with uniform and continuous distribution, which will improve the coercivity during the annealing process. This method can be widely used in the preparation and production of low weight rare earth high performance sintered NdFeB.

### IMPLEMENTING EXAMPLE 1

The main alloy composition is (Pr₂Nd₈)₃₀Fe_{bal}B_{0.95}(CoCuAlGa)₂ and the auxiliary alloy composition is (Pr₂Nd₈)₄₀Fe_{bal}B_{0.3}(CoCuAlGaTi)₃ and the alloy flakes are obtained by a convetional strip casting process. The main alloy flakes and the auxiliary alloy flakes are mixed in proportion ratio of 9 to 1. The mixed flakes are put into a hydrogen treatment furnace for conventional hydrogen absorption and dehydrogenation. The obtained alloy pieces are mixed with an antioxidant and a lubricant, and is crushed into a powder by jet milling, wherein the powder has an average particle size D50 of 3.8µm. A Dy powder having an average the particle size of 1.5µm is added to the milled powder with a mass percentage rate of 0.5wt% and the composition is mixed uniformly in a three-dimensional mixing machine for about 90 to 150min. The mixed powder is pressed to a green compact while applying a magnetic field of 2.0T. The green compact is put into a vacuum furnace to perform a thermal treatment including a sintering step and an annealing step. The sintering step is performed at 1050°C for 6 hours. The annealing step is perfomed at 850°C for 3hours, and then the temperature is reduced to 500°C for 3 hours.

### IMPLEMENTING EXAMPLE 2

The preparation conditions are the same as in Implementing Example 1 except that the main alloy composition is (Pr₂Nd₈)₃₀Fe_{bal}B_{0.95}(CoCuAlGa)₂ and the auxiliary alloy composition is (Pr₂Nd₈)₄₀Fe_{bal}(CoCuAlGaTi)₃.

### IMPLEMENTING EXAMPLE 3

The preparation conditions are the same as in Imlementing Example 1 except that the main alloy composition is (Pr₂Nd₈)₃₀Fe_{bal}B_{0.95}(CoCuAlGa)₂ and the auxiliary alloy composition is (Pr₂Nd₈)₄₀Fe_{bal}B_{0.3}(CoCuAlGaTi)₃. Further, the Dy powder is added with an amount of 1.0wt.%

### IMPLEMENTING EXAMPLE 4

The preparation conditions are the same as in Implementing Example 1 except that the main alloy composition is (Pr₂Nd₈)₃₀Fe_{bal}B_{0.95}(CoCuAlGa)₂ and the auxiliary alloy composition is (Pr₂Nd₈)₄₀Fe_{bal}B_{0.3}(CoCuAlGaTi)₃. Further, 0.5wt.% of a Tb powder with an average particle size of 1.0µm instead of the Dy powder is added.

### IMPLEMENTING EXAMPLE 5

The preparation conditions are the same as in Implementing Example 1 except that the main alloy composition is (Pr₂Nd₈)₃₀Fe_{bal}B_{0.95}(CoCuAlGa)₂ and the auxiliary alloy composition is Pr₄₀Fe_{bal}B_{0.3}(CoCuAlGaTi)₃.

### IMPLEMENTING EXAMPLE 6

The preparation conditions are the same as in Implementing Example 1 except that the main alloy composition is (Pr₂Nd₈)₃₀Fe_{bal}B_{0.95}(CoCuAlGa)₂ and the auxiliary alloy composition is Nd₄₀Fe_{bal}B_{0.3}(CoCuAlGaTi)₃.

### IMPLEMENTING EXAMPLE 7

The preparation conditions are the same as in Implementing Example 1 except that the main alloy composition is (Pr₂Nd₈)₃₀Fe_{bal}B_{0.95}(CoCuAlGa)₂ and the auxiliary alloy composition is (Pr₅Nd₅)₄₀Fe_{bal}B_{0.3}(CoCuAlGaTi)₃.

### COMPARATIVE EXAMPLE 1

The NdFeB alloy composition is (Pr₂Nd₈)_{30.5}Fe_{bal} B_{0.9}(CoCuAlGa)₂ and made into alloy flakes by a strip casting process. The alloy flakes are put into a hydrogen treatment furnace for conventional hydrogen absorption and dehydrogenation. The obtained alloy pieces are mixed with an antioxidant and a lubricant, and are crushed into a powder by jet milling with an average particle size of 3.8µm. The milled powder is pressed to a green compact while applying a magnetic field of 2.0T. The green compact is put into a vacuum furnace to get the magnet. The sintering process is performed at 1050°C for 6 hours, and the annealing treatment is performed at 850°C for 3hours, and then the temperature is reduced to 500°C for 3 hours.

### COMPARATIVE EXAMPLE 2

The main alloy composition is (Pr₂Nd₈)₃₀Fe_{bal}B_{0.95}(CoCuAlGa)₂ and the auxiliary alloy composition is (Pr₂Nd₈)₄₀Fe_{bal}B_{0.3}(CoCuAlGaTi)₃ are alloy flakes are made by a strip casting process. The main alloy flakes and the auxiliary alloy flakes are mixed in proportion ratio of 9 to 1, and the mixed flakes are put into a hydrogen treatment furnace for conventional hydrogen absorption and dehydrogenation. The obtained alloy pieces are mixed with an antioxidant and lubricant, and are crushed into a powder by jet milling with an average particle size of 3.8µm. The mixed powders are pressed to a green compact while applying a magnetic field of 2.0T. The green compact is put into a vacuum furnace to get the magnet. The sintering process is performed at 1050°C for 6 hours. The annealing treatment is performed at 850°C for 3hours and then the temperature is reduced to 500°C for 3 hours.

Process parameters and magenetic characteristics of Implementing Examples 1 to 7 and Comparative Examples 1 and 2 are listed in Table 1.

**Table 1: process parameters of the examples**

| | B content of auxiliary alloy | Rare earth type of auxiliary alloy | Adding rate of auxiliary alloy | Adding of heavy rare earth powder | Br (T) | Hcj (kA/m) |
|---|---|---|---|---|---|---|
| Implementing example 1 | 0.3wt% | Pr₂Nd₈ | 10% | Dy powder:0.5wt.% powder size:1.5µm | 1.430 | 1393 |
| Implementing example 2 | 0wt% | Pr₂Nd₈ | 10% | Dy powder:0.5wt.% powder size:1.5µm | 1.433 | 1385 |
| Implementing example 3 | 0.3wt% | Pr₂Nd₈ | 10% | Dy powder:1.0wt.% powder size:1.5µm | 1.425 | 1457 |
| Implementing example 4 | 0.3wt% | Pr₂Nd₈ | 10% | Tb powder:0.5wt.% powder size:1.0µm | 1.435 | 1473 |
| Implementing example 5 | 0.3wt% | Pr | 10% | Dy powder 0.5wt.% powder size:1.5µm | 1.428 | 1427 |
| Implementing example 6 | 0.3wt% | Nd | 10% | Dy powder 0.5wt.% powder size:1.5µm | 1.433 | 1399 |
| Implementing example 7 | 0.3wt% | Pr₅Nd₅ | 10% | Dy powder 0.5wt.% powder size:1.5µm | 1.430 | 1411 |
| Comparative example 1 | No adding auxiliary alloy | Pr₂Nd₈ | No adding | 0 | 1.440 | 1114 |
| Comparative example 2 | 0.3wt% | Pr₂Nd₈ | 10% | 0 | 1.440 | 1274 |

Compared with Comparative Example 1, the Implementing Examples 1 to 4 show improved coercivity by adding the auxiliary alloy with the rare earth elements Pr₂Nd₈. Compared with the Comparative Example 2 where no heavy rare earth powder is added, the Implementing Examples 1 to 3 show an improved magnetic coercivity. Comparing Implementing Examples 5 to 6 with Comparative Example 1, shows that adjusting the ratio of Pr and Nd of the auxiliary alloy also can improve the coercivity, especially when Pr and Nd metal are both selected, the improvement effect of coercivity is more obvious when the content of Pr increases.

The preparation method only uses a low amount of added heavy rare earth powder to improve the properties of the sintered NdFeB magnet. Due to the use of an auxiliary alloy, the formation of the grain boundary phase is improved and the heavy rare earth elements Dy or Tb are carried by the lower melting auxiliary alloy resulting in an evenly dispersion of the heavy rare earth metals around the main phase. Under the sintered temperature, the Dy or Tb will diffuse into the surface layer of the main phase, forming the desired DyFeB or TbFeB phase with high H_{A}. Thereby, the coercivity can be significantly improved and remanence kept high.

## Claims

1. A preparation method for NdFeB permanent magnet, the method including the steps of:
a) Preparing main alloy flakes consisting of (Pr₂Nd₈)ₓFe_{100-x-y-z}B_{y}M_{z}, where M is at least one of Al, Co, Cu, Ga, Ti and Zr, and x, y and z is 28.5wt.%≤x≤31.0wt.%, 0.85wt.%≤y≤0.98wt.% and 0.5wt.%≤z≤5.0wt.%;
b) Preparing auxiliary alloy flakes consisting of LᵤFe_{100-u-v-w}BᵥM_{w}, where L is one or more of the metals Pr and Nd, M is at least one of Al, Co, Cu, Ga, Ti and Zr, and u, v and w is 35.0 wt.%≤u≤45.0wt.%, 0wt.%≤v≤5.0wt.% and 2.0wt.%≤w≤10.0wt.%;
c) Mixing the main alloy flakes and the auxiliary alloy flakes in a predetermined rate, then performing a hydrogen decrepitation to produce alloy pieces, and then crushing the alloy pieces to an alloy powder by jet milling;
d) Preparing a powder mixture including the alloy powder and an added heavy rare earth powder consisting of at least one of Dy and Tb; and
e) Pressing the powder mixture to a green compact while applying a magnetic field, and thermal treatment of the green compact in a vacuum furnace to obtain the NdFeB permanent magnet.

2. The preparation method of claim 1, wherein the auxiliary alloy includes Pr and Nd.

3. The preparation method of claim 2, wherein a content ratio of Pr to Nd is in the range of 0.25 to 1.

4. The preparation method of any one of the preceding claims, wherein the auxiliary alloy flakes are added in proportion of 5wt% to 20wt% in step c).

5. The preparation method of any one of the preceding claims, wherein the heavy rare earth powder, which is added in step d), has an average particle size D50 in the range of 1.0µm-3.0µm, the mass percentage of the heavy rare earth is in the range of 0.05% to 1.0%, and the powder are mixed about 90 to 150min.

6. The preparation method of any one of the preceding claims, wherein the thermal treatment of step e) includes a sub-step of sintering the green compact at a temperature in the range of 850°C to 950°C for 2 to 5 hours, and then heating to 1030°C to1090°C for 4 to 8h.

7. The preparation method of claim 6, wherein the thermal treatment of step e) further includes the sub-steps of cooling the sintered green compact, and then annealing the sintered compact at a temperature in the range of 800°C to 900°C for 2 to 4 hours and then at a temperature in the range of 450°C to 550°C for 3 to 6 hours.

## Patentansprüche

1. Verfahren zur Herstellung eines NdFeB-Permanentmagneten, wobei das Verfahren die folgenden Schritte umfasst:
a) Herstellen von Hauptlegierungsflocken, bestehend aus (Pr₂Nd₈)ₓFe_{100-x-y-z}B_{y}M_{z}, wobei M mindestens eines von Al, Co, Cu, Ga, Ti und Zr ist und x, y und z 28,5 Gew.-%≤x≤31,0 Gew.-%, 0,85 Gew.-%≤y≤0,98 Gew.-% und 0,5 Gew.-%≤z≤5,0 Gew.-% betragen;
b) Herstellen von Hilfslegierungsflocken, bestehend aus LᵤFe_{100-u-v-w}BᵥM_{w}, wobei L eines oder mehrere der Metalle Pr und Nd ist, M mindestens eines von Al, Co, Cu, Ga, Ti und Zr ist und u, v und w 35,0 Gew.-%≤u≤45,0Gew.-%, 0Gew.-%≤v≤5,0Gew.-% und 2,0Gew.- %≤w≤10,0Gew.-% sind;
c) Mischen der Hauptlegierungsflocken und der Hilfslegierungsflocken in einem vorbestimmten Verhältnis, dann Durchführen einer Wasserstoffdekrepitation, um Legierungsstücke zu erzeugen, und dann Zerkleinern der Legierungsstücke zu einem Legierungspulver durch Strahlmahlen;
d) Herstellen einer Pulvermischung, die das Legierungspulver und ein zugesetztes schweres Seltenerdpulver enthält, das aus mindestens einem von Dy und Tb besteht; und
e) Pressen der Pulvermischung zu einem Grünling unter Anlegen eines Magnetfeldes und thermische Behandlung des Grünlings in einem Vakuumofen zur Gewinnung des NdFeB-Permanentmagneten.

2. Herstellungsverfahren nach Anspruch 1, wobei die Hilfslegierung Pr und Nd enthält.

3. Herstellungsverfahren nach Anspruch 2, wobei ein Gehaltsverhältnis von Pr zu Nd im Bereich von 0,25 bis 1 liegt.

4. Herstellungsverfahren nach einem der vorhergehenden Ansprüche, wobei die Hilfslegierungsflocken in Schritt c) in einem Anteil von 5 Gew.-% bis 20 Gew.-% zugesetzt werden.

5. Herstellungsverfahren nach einem der vorhergehenden Ansprüche, wobei das schwere Seltenerdpulver, das in Schritt d) zugegeben wird, eine durchschnittliche Teilchengröße D50 im Bereich von 1,0 µm bis 3,0 µm aufweist, der Massenprozentsatz der schweren Seltenen Erde im Bereich von 0,05 % bis 1,0 % liegt und das Pulver etwa 90 bis 150 Minuten gemischt wird.

6. Herstellungsverfahren nach einem der vorhergehenden Ansprüche, wobei die thermische Behandlung von Schritt e) einen Unterschritt des Sinterns des Grünlings bei einer Temperatur im Bereich von 850°C bis 950°C für 2 bis 5 Stunden und dann ein Erhitzen auf 1030°C bis 1090°C für 4 bis 8 Stunden umfasst.

7. Herstellungsverfahren nach Anspruch 6, wobei die thermische Behandlung von Schritt e) ferner die Unterschritte des Abkühlens des gesinterten Grünlings und des anschließenden Glühens des Sinterlings bei einer Temperatur im Bereich von 800°C bis 900°C für 2 bis 4 Stunden und dann bei einer Temperatur im Bereich von 450°C bis 550°C für 3 bis 6 Stunden umfasst.

## Revendications

1. Procédé de préparation d'un aimant permanent en NdFeB, le procédé comprenant les étapes suivantes :
a) préparation de flocons d'alliage principal constituées de (Pr₂Nd₈)ₓFe_{100-x-y-z}B_{y}M_{z}, où M est au moins l'un de AI, Co, Cu, Ga, Ti et Zr, et où x, y et z représentent 28,5 % en poids≤x≤31,0 % en poids, 0,85 % en poids≤y≤0,98 % en poids et 0,5 % en poids≤z≤5,0 % en poids ;
b) préparation de flocons d'alliage auxiliaire constituées de LᵤFe_{100-u-v-w}BᵥM_{w}, où L est un ou plusieurs des métaux Pr et Nd, M est au moins l'un de AI, Co, Cu, Ga, Ti et Zr, et u, v et w est 35,0 % en poids≤u≤45, 0 % en poids≤v≤5,0 % en poids et 2,0 % en poids≤w≤10,0 % en poids ;
c) mélange des flocons d'alliage principal et des flocons d'alliage auxiliaire à un taux prédéterminé, puis exécution d'une décrépitation à l'hydrogène pour produire des pièces d'alliage, et enfin broyage des pièces d'alliage pour obtenir une poudre d'alliage par broyage à jet ;
d) préparation d'un mélange de poudres comprenant la poudre d'alliage et une poudre de terre rare lourde ajoutée consistant en au moins l'un de Dy et Tb ; et
e) pressage du mélange de poudres en un compact vert tout en appliquant un champ magnétique, et traitement thermique du compact vert dans un four sous vide pour obtenir l'aimant permanent en NdFeB.

2. Procédé de préparation de la revendication 1, dans lequel l'alliage auxiliaire comprend du Pr et du Nd.

3. Procédé de préparation de la revendication 2, dans lequel le rapport entre la teneur en Pr et en Nd est compris entre 0,25 et 1.

4. Procédé de préparation de l'une quelconque des revendications précédentes, dans lequel les flocons d'alliage auxiliaire sont ajoutées dans une proportion de 5% en poids à 20% en poids à l'étape c).

5. Procédé de préparation de l'une quelconque des revendications précédentes, dans lequel la poudre de terre rare lourde, qui est ajoutée à l'étape d), a une taille de particule moyenne D50 comprise entre 1,0µm-3,0µm, le pourcentage massique de la terre rare lourde étant compris entre 0,05% et 1,0%, et la poudre étant mélangée environ 90 à 150min.

6. Procédé de préparation selon l'une quelconque des revendications précédentes, dans lequel le traitement thermique de l'étape e) comprend une sous-étape de frittage du compact vert à une température comprise entre 850°C et 950°C pendant 2 à 5 heures, puis un chauffage à 1030°C à1090°C pendant 4 à 8h.

7. Procédé de préparation selon la revendication 6, dans lequel le traitement thermique de l'étape e) comprend en outre les sous-étapes consistant à refroidir le compact vert fritté, puis à recuire le compact fritté à une température comprise entre 800°C et 900°C pendant 2 à 4 heures, puis à une température comprise entre 450°C et 550°C pendant 3 à 6 heures.
